# NEW EUROPEAN PATENT SPECIFICATION

(11) **EP 1 512 736 B2**
(45) Date of publication and mention of the opposition decision: **17.12.2025**
(45) Mention of the grant of the patent: 02.05.2018
(21) Application number: 04255073.1
(22) Date of filing: 24.08.2004
(51) Int. Cl.: C10L 1/10, C10L 1/12, C10L 1/18, C10L 1/188, C10L 1/19, C10L 1/196, C10L 1/198, C10L 1/224, C10L 1/236, C10L 10/06, C10L 10/08, C10L 10/14, C10L 10/18

(54) **Stabilised diesel fuel additive compositions**
Stabilisierte Additivzusammensetzungen für Dieselkraftstoffe
Compositions d'additifs stabilisées pour carburants diesel

(30) Priority: 05.09.2003 EP 03255551
(43) Date of publication of application: 09.03.2005
(73) Proprietor: Infineum International Limited, Abingdon, Oxfordshire OX13 6BB (GB)
(72) Inventor: Caprotti, Rinaldo, Oxford Oxfordshire, OX2 9HD (GB); Thompson, Russell Martin, North Leigh Witney Oxford, OX29 6TT (GB)
(74) Representative: Eisenführ Speiser

(56) References cited:
- EP-A1- 1 344 809
- EP-A2- 0 671 205
- WO-A1-87/05924
- WO-A2-02/02720
- CA-A- 970 553
- FR-A1- 2 768 155
- FR-A1- 2 789 601
- FR-A5- 2 097 879
- GB-A- 2 248 068
- US-A- 3 272 746
- US-A- 3 438 756

## Description

This invention relates to novel fuel additive compositions. More particularly, this invention relates to fuel compositions containing metallic additives which are stabilised against phase separation. Metallic additives are added to fuels since they are especially effective in improving the performance of particulate traps which are used in the exhaust systems of diesel engines, amongst other uses.

Diesel engines equipped with particulate traps, mounted in the exhaust stream, to "trap" or collect particulates in the exhaust to prevent their emission to the atmosphere are expected to be in greater use in the next few years.

Diesel engines running without particulate traps emit unburned hydrocarbons (HC), carbon monoxide (CO), nitrogen oxides (NOₓ), and particulates, all of which are subject to current or proposed regulation. The problems of controlling these pollutants are compounded because there is a trade-off between particulates and nitrogen oxides: when the combustion conditions are modified to favor low nitrogen oxides emissions, particulates are increased. Particulate traps are employed to reduce the severity of the particulate emissions.

Diesel particulates, their effect and control, are at the center of much concern and controversy. Their chemistry and environmental impact present complex issues. Generally, the diesel particulate matter is principally solid particles of carbon and metal compounds with adsorbed hydrocarbons, sulphates and aqueous species. Among the adsorbed species are aldehydes and polycyclic aromatic hydrocarbons. Some of these organics have been reported to be potential carcinogens or mutagens. Unburned hydrocarbons are related to the characteristic diesel odour and include aldehydes such as formaldehyde and acrolein. The need to control nanoparticles is likely to lead to mandates requiring traps.

The use of diesel traps and the need to improve them has resulted in a great deal of research and a great number of patents and technical publications. The traps are typically constructed of metal or ceramic and are capable of collecting the particulates from the exhaust and withstanding the heat produced by oxidation of carbonaceous deposits which must be burned off at regular intervals.

This burning off, or regeneration, could occur by itself if the operating temperature of the trap were sufficiently high. However, in the typical situation, the exhaust temperature is not constantly high enough, and secondary measures such as electrically heating to raise the trap temperature or using a catalyst on the washcoat to reduce the combustion temperature of particulates, have not been fully successful.

The use of organometallic salts and complexes to improve the operation of diesel engine particulate traps is disclosed, for example, in U.S. Patent No. 5,344,467 issued September 6, 1994, which teaches the use of a combination of an organometallic complex and an antioxidant. The organometallic complex is soluble or dispersible in the diesel fuel and is derived from an organic compound containing at least two functional groups attached to a hydrocarbon linkage.

WO 99/36488 published July 22, 1999 discloses fuel additive compositions which contain at least one iron-containing fuel-soluble or fuel-dispersible species in synergistic combination with at least one alkaline earth group metal-containing fuel-soluble or fuel-dispersible species. This combination of metallic additives is said to improve the operation of the diesel particulate filter traps.

WO 94/11467 published May 26, 1994 teaches a method to improve the operation of diesel traps through the use of a fuel additive comprising fuel-soluble compositions of a platinum group metal in effective amounts to lower the emissions of unburned hydrocarbons and carbon monoxide from the trap. The platinum group metals comprise platinum, palladium, rhodium or iridium.

Co-pending European application EP-A-1 344 809 describes a diesel fuel composition which improves the diesel engine particulate traps, comprising a metal salt-ashless detergent additive combination effective in improving the performance of the particulate trap. A wide variety of metals are disclosed, in the context of organo-metallic salts.

US-A-3,438,756 describes barium compounds provided to fuels to reduce smoking and comprising the reaction product of alkylphenol with a relatively high molecular weight alkenyl succinic acid and barium carbonate, prepared by carbonation of barium oxide dispersed in the presence of the alkyl phenol and alkenyl succinic acid.

EP 671205, EP 599717 and EP 575189 disclose the use of various cerium compounds in fuels.

A problem observed in connection with the formulation of diesel fuels having solubilised or colloidally dispersed metals such as metal oxides is the tendency to undergo phase separation upon storage, as evidenced by formation of haze or actual separation of layers. This problem is even more pronounced in connection with low sulphur diesel fuels which also contain a variety of additives.

The present invention is based upon a discovery that such fuels may be stabilised against such phase separation or haze formation by the addition of very small amounts of an oil-dispersible or oil-soluble compound having two or more contiguous polar head groups.

In accordance with this invention there have been discovered diesel fuel compositions stabilised against phase separation comprising a diesel fuel, a colloidally dispersed or solubilised metal catalyst compound for diesel particulate trap regeneration and an oil soluble or oil dispersible organic compound having a lipophilic hydrocarbyl chain having attached directly thereto at least two contiguous polar head functional groups, the organic compound being present in an amount effective to stabilise the metal catalyst compound against phase separation, wherein the metal catalyst compound consists of cerium or iron oxides or mixtures thereof, and wherein the composition of the invention is further particularised in claim 1.

The organic compound is generally present in an amount of 10 to 1,000 ppm, preferably 10 to 200 ppm, most preferably 10 to 50 ppm (weight) of compound per weight of diesel fuel composition in order to effectively stabilise the metal catalyst compound.

In this specification, the term 'contiguous polar head functional groups' is used to represent polar (functional chemical) groups which are separated by no more than three, preferably no more than two carbon atoms within the molecule.

The invention is particularly applicable to diesel fuel compositions which contain as catalysts for diesel particulate trap regeneration effective amounts of metallic compounds, typically sufficient to provide 1 to 200, 1 to 100, 1 to 20, 1 to 10, or 1 to 5 ppm metal (by weight) in the fuel, in the form of colloidally dispersed or solubilised compounds.

The composition's metal catalyst compound consists of cerium or iron oxides or mixtures thereof.

The stabiliser compound of the present invention is represented by the generalised formula A-C-B, where C represents a hydrocarbyl chain of Mn (number average molecular weight) 200 - 4,000, preferably 200 - 1,300, more preferably 200 - 1,000 such as 400 - 1,000, 700-1000 or 450 - 700.

The stabilisers may also be described in the following pictorial representation:

In the formula above, n may be 1-20, but is preferably 1-10, more preferably 1-5. When n is greater than 1, the stabiliser includes compounds of the following formulas, where "PIB" is polyisobutenyl, "PIBSA" is polyisobutenyl succinic anhydride and R is the lipophilic hydrocarbyl group: Hydrolysed poly(PIBSA) Hydrolysed alternating copolymers of (alpha-olefin-*alt*-maleic anhydride)

This hydrocarbyl chain may be straight or branched, but branched hydrocarbyl chains are preferred because of their increased degree of solubility and preferably the hydrocarbyl chain is a polyisobutenyl group in the molecular weight ranges given above. In the aforesaid formula A and B represent at least two contiguous carboxylate residues attached directly to one end of the lipophilic C chain, , being either groups of the formula -COOH or ionized as -(COO⁻)ₙMⁿ⁺ where M is a quaternary ammonium cation. Typical examples of suitable quaternary ammonium cations are the ammonium ion itself, NH₄⁺, and the following quaternary ammonium cations R₄N⁺, R₃NH⁺, R₂NH₂⁺, RNH₃⁺ derived from tertiary, secondary and primary amines respectively where R = H or a straight or branched alkyl chain or aromatic moiety containing from 1 to 22 carbon atoms.

Compounds with two contiguous groups that are capable of binding or otherwise coordinating to a metal or metal oxide moiety are known in the art as bidentate. By varying the nature of the carboxylate derivative used, the head grouping can be made to be tridentate, tetradentate and polydentate in surface binding ability.

Particularly preferred stabiliser additives for use in the composition of the present invention are polyisobutenyl succinic acid wherein the polyisobutenyl group has a Mn of 1,000, and polyisobutenyl succinic acid wherein the polyisobutenyl group has a molecular weight of 450.

Further embodiments of this invention comprise fuel compositions comprising the stabiliser compound, metal catalyst compound and one or more other fuel additive compounds, such as a lubricity enhancing additive, diesel detergent additive or a cold flow additive.

Still further embodiments comprise additive concentrate compositions containing 3 to 75 % by weight of the stabiliser of this invention, in combination with the particulate trap metal catalyst compound, optionally in further combination with one or more other fuel additive compounds selected from other lubricity-enhancing compounds; cold flow improvers such as ethylene-unsaturated ester copolymers, hydrocarbon polymers, polar nitrogen compounds, alkylated aromatics, linear polymer compounds and comb polymers; detergents; corrosion inhibitors; dehazers; demulsifiers; metal deactivators; antifoaming agents; combustion improvers such as cetane improvers; package compatibilisers; reodorants; metallic-based additives such as metallic combustion improvers; dyes; bacteriostatic agents; gum inhibitors; upper cylinder lubricants and anti-icing agents and antioxidants.

A concentrate comprising the additive dispersed in carrier liquid (e.g. in solution) is convenient as a means of incorporating the additive. The concentrates of the present invention are convenient as a means for incorporating the additive into bulk oil such as distillate fuel, which incorporation may be done by methods known in the art. The concentrates may also contain other additives as required and preferably contain from 3 to 75 wt %, more preferably 3 to 60 wt %, and most preferably 10 to 50 wt % of the additive or additives preferably in solution in oil. Examples of carrier liquid are organic solvents including hydrocarbon solvents, for example petroleum fractions such as naphtha, kerosene, diesel and heater oil; aromatic hydrocarbons such as aromatic fractions, e.g. those sold under the 'SOLVESSO' trade name; alcohols and/or esters; and paraffinic hydrocarbons such as hexane and pentane and isoparaffins. Higher boiling paraffinic liquids are preferred. Alkylphenols, such as nonylphenol and 2,4-di-t-butylphenol either alone or in combination with any of the above have also been found to be particularly useful as carrier solvents. The carrier liquid must, of course, be selected having regard to its compatibility with the additive and with the fuel.

Further embodiments of the invention include :
the use, in a diesel fuel composition comprising a diesel fuel and the colloidally dispersed or solubilised metal catalyst compound as defined above, of the oil soluble or oil dispersible organic compound defined above to reduce the tendency of the diesel fuel and the colloidally dispersed or solubilised metal catalyst compound to form separate phases within the diesel fuel composition over time;
the use of the oil soluble or oil dispersible organic compound defined above, in an additive concentrate comprising the metal catalyst compound defined above, to improve the colloidal dispersability or solubility of the metal catalyst compound in diesel fuel; and
a process for enhancing the oil dispersibility or solubility of the metal catalyst compound defined above, comprising the addition thereto of the oil soluble or oil dispersible organic compound defined above to a diesel fuel composition comprising a diesel fuel and the metal catalyst compound.

Examples of other stabiliser compounds are as follows wherein R is hydrocarbyl:
the acylated aspartic and glutamic acid moieties
Glutamic acid derivatives are examples of the present invention where the contiguous polar head groups (COOH) are separated in space by three carbon atoms.

The fuel oil may be a petroleum-based fuel oil, suitably a middle distillate fuel oil, i.e. a fuel oil obtained in refining crude oil as the fraction between the lighter kerosene and jet fuels fraction and the heavy fuel oil fraction. Such distillate fuel oils generally boil above about 100°C. The fuel oil can comprise atmospheric distillate or vacuum distillate, or cracked gas oil or a blend in any proportion of straight run and thermally and/or catalytically cracked and/or hydroprocessed distillates. The most common petroleum-based fuel oils are kerosene, jet fuels and preferably diesel fuel oils.

The sulphur content of the fuel oil may be 2000 or less, preferably 500 or less, more preferably 50 or less, most preferably 10 or less, ppm by mass based on the mass of the fuel oil. The art describes methods for reducing the sulphur content of hydrocarbon middle distillate fuels, such methods including solvent extraction, sulphuric acid treatment, and hydrodesulphurisation.

Preferred fuel oils have a cetane number of at least 40, preferably above 45 and more preferably above 50. The fuel oil may have such cetane numbers prior to the addition of any cetane improver or the cetane number of the fuel may be raised by the addition of a cetane improver.

Advantageously, the fuel oils are those that have low solvency properties caused by low aromatic concentrations (e.g. below 30, below 20, below 15, below 10, or below 5, mass per cent), and/or those that are required to operate at low temperatures such as at -5, -10, -15, or -20, °C or lower.

Other examples of fuel oils include jet-fuels; Fischer-Tropsch fuels; biofuels such as fuels made from vegetable matter such as rape seed methyl ester; and diesel/alcohol or diesel/water emulsions or solutions. Fischer-Tropsch fuels, also known as FT fuels, include those that are described as gas-to-liquid fuels and coal conversion fuels. To make such fuels, syngas (CO + H₂) is first generated and then converted to normal paraffins by a Fischer-Tropsch process. The normal paraffins may then be modified by processes such as catalytic cracking/reforming or isomerisation, hydrocracking and hydroisomerisation to yield a variety of hydrocarbons such as iso-paraffins, cyclo-paraffins and aromatic compounds. The resulting FT fuel can be used as such or in combination with other fuel components and fuel types such as those mentioned in this specification. Also suitable are fuels emulsified with water and alcohols, which contain suitable surfactants, and residual fuel oil used in marine diesel engines. WO-A- 0104239; WO-A- 0015740; WO-A-0151593; WO-A- 9734969; and WO-155282 describe examples of diesel/water emulsions. WO-A- 0031216; WO-A- 9817745; and WO-A- 024 8294 describe examples of diesel-ethanol emulsions/mixtures.

Preferred vegetable-based fuel oils are triglycerides of monocarboxylic acids, and these typically have the general formula shown below where R is an aliphatic radical of 10-25 carbon atoms which may be saturated or unsaturated.

Generally, such oils contain glycerides of a number of acids, the number and kind varying with the source vegetable of the oil. Suitable fuel oils also include mixtures of 1-100% by weight of vegetable oils or methylesters of fatty acid, with petroleum based diesel fuel oils.

Examples of oils and methyl ester derived fuel are tall oil, rapeseed oil, coriander oil, soyabean oil, cottonseed oil, sunflower oil, castor oil, olive oil, peanut oil, maize oil, almond oil, palm kernel oil, coconut oil, mustard seed oil, beef tallow and fish oils. Rapeseed oil, which is a mixture of fatty acids esterified with glycerol, is preferred as it is available in large quantities and can be obtained in a simple way by pressing from rapeseed.

Further preferred examples of vegetable-based fuel oils are alkyl esters, such as methyl esters, of fatty acids of the vegetable or animal oils. Such esters can be made by transesterification.

As lower alkyl esters of fatty acids, consideration may be given to the following, for example as commercial mixtures containing, for example: the ethyl, propyl, butyl and especially methyl esters of fatty acids with 12 to 22 carbon atoms, for example, mixtures of lauric acid, myristic acid, palmitic acid, palmitoleic acid, stearic acid, oleic acid, elaidic acid, petroselic acid, ricinoleic acid, elaeostearic acid, linoleic acid, linolenic acid, eicosanoic acid, gadoleic acid, docosanoic acid or erucic acid, and rosin acid and isomers which have an iodine number from 50 to 180, especially 90 to 180. Mixtures with particularly advantageous properties are those which contain mainly, i.e. to at least 50 wt % methyl esters of fatty acids with 16 to 22 carbon atoms and 1, 2 or 3 double bonds. The preferred lower alkyl esters of fatty acids are the methyl esters of oleic acid, linoleic acid, linolenic acid and erucic acid.

Commercial mixtures of the stated kind are obtained for example by cleavage and esterification of natural fats and oils by their transesterification with lower aliphatic alcohols. For production of lower alkyl esters of fatty acids it is advantageous to start from fats and oils with high iodine number, such as, for example, sunflower oil, rapeseed oil, coriander oil, castor oil, soyabean oil, cottonseed oil, peanut oil or beef tallow. Lower alkyl esters of fatty acids based on a new variety of rapeseed oil, the fatty acid component of which is derived to more than 80 wt % from unsaturated fatty acids with 18 carbon atoms, are preferred.

Most preferred as a vegetable-based fuel oil is rapeseed methyl ester.

Where the fuel comprises the above-defined biofuels (either alone, or in combination with other fuels from other sources, such as petroleum-based fuels), it has been found that higher proportions of the stabiliser compound can be required to impart effective stability against phase separation. Thus, in such embodiments, the amount of the stabiliser compound should typically exceed 20 ppm weight (per weight of fuel), more preferably 25 to 200 ppm of stabiliser compound. This effect is particularly prevalent with lower alkyl esters of fatty acids, such as rapeseed and other vegetable oil methyl esters.

The fuel compositions of the invention may additionally comprise one or more other fuel additives, or co-additives, as indicated above. Examples include other lubricity-enhancing compounds; cold flow improvers such as ethylene-unsaturated ester copolymers, hydrocarbon polymers, polar nitrogen compounds, alkylated aromatics, linear polymer compounds and comb polymers; detergents; corrosion inhibitors (anti-rust additives); dehazers; demulsifiers; metal deactivators; antifoaming agents; combustion improvers such as cetane improvers; co-solvents; package compatibilisers; reodorants; and metallic-based additives such as metallic combustion improvers.

The inventive diesel fuel compositions can contain other fuel additives which are well known to those of skill in the art. These include dyes, cetane improvers, rust inhibitors such as alkylated succinic acids and anhydrides, bacteriostatic agents, gum inhibitors, metal deactivators, demulsifiers, upper cylinder lubricants and anti-icing agents and antioxidants.

Stabilised compositions of this invention will preferably contain one or more of the various lubricity additives which are now commonly used in low sulphur fuels, i.e., fuels having less than 0.2 wt % sulphur, preferably less than 0.1 wt % such as 0.005 or 0.001 wt % sulphur or less. Such lubricity additives include monohydric or polyhydric alcohol esters of C₂-C₅₀ carboxylic acids such as glycerol monooleate, esters of polybasic acids with C₁-C₅ monohydric alcohols, esters of dimerized carboxylic acids, reaction products of polycarboxylic acids and epoxides such as 1,2-epoxyethane and 1,2-epoxypropane and lubricity additives derived from fatty acids such as vegetable oil fatty acid methyl esters, as well as fatty acid amides of monoethanolamine and diethanolamine.

Further examples are lubricity additives prepared by combining the aforesaid esters of C₂-C₅₀ carboxylic acids with an ashless dispersant comprising an acylated nitrogen compound having a hydrocarbyl substituent of at least 10 carbon atoms made by reacting an acylating agent with an amino compound, such as the reaction products of polyisobutenyl (C₈₀-C5₀₀) succinic anhydride with ethylene polyamines having 3 to 7 amino nitrogen atoms.

Another example of lubricity additive chemistry are compounds of the following formula, described in WO 97/45507 and WO 02/02720: Where R¹ is a C₁₀₋₃₂ alkenyl group and R² and R³ are (-OCH₂CH₂)ₙOH, (-OCH₂CHCH₃)ₙOH, or -OCH₂CHOHCH₂OH in which n = 1-10.

Other lubricity additives are combinations of the aforesaid esters with ethylene-unsaturated ester copolymers having, in addition to units derived from ethylene, units of the formula

-CR¹R²-CHR³-

wherein R¹ represents hydrogen or methyl; R² represents COOR⁴, wherein R⁴ represents an alkyl group having from 1 to 9 carbon atoms which is straight chain or, if it contains 2 or more carbon atoms, branched, or R² represents OOCR⁵, wherein R⁵ represents R⁴ or H; and R³ represents H or COOR⁴. Examples are ethylene-vinyl acetate and ethylene-vinyl propionate and other copolymers where there is present 5-40% of the vinyl ester.

As an alternative to the above described esters, or in combination therewith, the lubricity additive may comprise one or more carboxylic acids of the types disclosed in relation to the ester lubricity additives. Such acids may be mono- or polycarboxylic, saturated or unsaturated, straight or branched chain and may be generalised by the formula R¹(COOH)ₓ where x is 1-4 and R¹ is a C₂ to C₅₀ hydrocarbyl. Examples are capric, lauric, myristic, palmitic, oleic, elaidic, palmitoleic, petaoselic, ricinoleic, linoleic, linolenic, eicosanic, tall oil fatty and dehydrated castor oil fatty acids, and rosin acids and isomers and mixtures thereof. The polycarboxylic acid may be a dimer acid such as that formed by dimerization of unsaturated fatty acids such as linoleic or oleic acid.

Other lubricity additives are hydroxy amines of the formula where R¹ is an alkenyl radical having one or more double bonds or an alkyl radical and containing from 4 to 50 carbon atoms, or a radical of the formula where each of R², R³, R⁴, R⁵, R⁶ and R⁷ is independently hydrogen or a lower alkyl radical; R⁸ is an alkenyl radical having one or more double bonds or an alkyl radical and containing from 4 to 50 carbon atoms; R⁹ is an alkylene radical containing from 2 to 35, e.g. 2 to 6, carbon atoms; each of p, q and v is an integer between 1 and 4; and each of a, b and c may be 0, providing that at least one of a, b or c is an integer between 1 and 75.

Other lubricity additives are ester, amine and amine salt derivatives of salicylic acid and alkylated salicylic acids.

The additives of the invention may also be used in combination with diesel performance additives such as silicon-containing anti-foam agents such as siloxane block copolymers or cetane improvers such as 2-ethyl hexyl nitrate.

The additives of the present invention may also be used in combination with an appropriate carrier liquid or organic solvent. Examples of carrier liquid are organic solvents including hydrocarbon solvents, for example petroleum fractions such as naphtha, kerosene, diesel and heater oil; aromatic hydrocarbons such as aromatic fractions, e.g. those sold under the 'SOLVESSO' tradename; paraffinic hydrocarbons such as hexane and pentane and isoparaffins, e.g., those sold under the 'ISOPAR' tradename; and oxygenated solvents such as alcohols. The carrier liquid must, of course, be selected having regard to its compatibility with the additive and with the fuel.

The stabiliser composition can be
1. Preferably added to the DPF (diesel particulate filter) additive composition prior to doping the mixture into the fuel.
2. Added to the fuel separately before or after addition of the DPF additive.
3. Added to any typical fuel additive composition, e.g., lubricity improver, detergent, cold flow improver, corrosion inhibitor, antistatic or mixtures thereof prior to doping the mixture into the fuel.
4. Added to the fuel separately before or after addition of any typical fuel additive composition.

The additive compositions of the invention, with or without diluent or solvent, may be incorporated into bulk fuel oil by methods such as those known in the art. If co-additives are required, they may be incorporated into the bulk fuel oil at the same time as the additives of the invention or at a different time.

The invention is further illustrated by the following examples.

### EXAMPLES

### Synthesis

### Example 1: Preparation of PIB₁₀₀₀ (polyisobutenyl Mn 1000) Succinic Acid (Invention) [Stabiliser A]

PIB₁₀₀₀SA (succinic anhydride) (10 g, 9.5 mmol), toluene (50 ml) and deionised water (15 ml, excess) were heated with stirring under reflux (∼85°C) for 6 hours.

After cooling, the organic phase was separated and dried over anhydrous MgSO₄. After filtration, the solvent was removed *in vacuo* at low temperature, giving a product which was used directly.
Infrared: v_{CO} 1714 (free acid) cm⁻¹.
%C, H, N: C, 80.8; H, 12.5; N, <0.1%.
TAV = 1.96 Meq/g; TAN = 110 mg KOH/g.

### Example 2: Preparation of Monoisopropyl Ester of PIB₁₀₀₀ Succinic Acid (Comparative) [Stabiliser B]

PIB₁₀₀₀SA (10 g, 9.5 mmol), toluene (50 ml) and isopropanol (50 ml, excess) were heated with stirring under reflux (∼85°C) for 6 hours.

After cooling, the solvent mixture was removed *in vacuo* at low temperature, giving a partially esterified product which was used directly.
Infrared: v_{CO} 1713 (free acid); 1734 (ester) cm⁻¹.
%C, H, N: C, 81.0; H, 12.5; N, 0.2%.
TAV = 1.37 Meq/g; TAN = 76 mg KOH/g.

### Example 3: Preparation of PIB₄₅₀ (polyisobutenyl Mn 450) Succinic Acid (Invention) [Stabiliser C]

PIB₄₅₀SA (50 g), Isopar L, a paraffinic solvent, (150 ml) and water (4 ml, excess) were heated with stirring under a reflux (∼120°C) for 12 hours.

After cooling, the organic phase was separated and dried over anhydrous MgSO₄. After filtration, the solvent mixture was removed *in vacuo* at low temperature, giving a product which was used directly.

The characteristics of the fuels tested are given below:

### Diesel Fuels used in Examples

### Diesel Fuel A: German Low Sulphur

| | |
|---|---|
| **CFPP (°C)** | -10 |
| **Cloud Point (°C)** | -9 |
| **Density @15 deg.C (kg/l)** | 0.827 |
| **Sulphur** | <10 ppm |

| **D86 Distillation (°C)** | |
|---|---|
| **IBP** | 179 |
| **10%** | 198 |
| **50%** | 248 |
| **95%** | 340 |
| **FBP** | 353 |

### Diesel Fuel B: German Low Sulphur

| | |
|---|---|
| **CFPP (°C)** | -9 |
| **Cloud Point (°C)** | -8 |
| **Density @15 deg.C (kg/l)** | 0.831 |
| **Sulphur** | <10 ppm |

| **D86 Distillation (°C)** | |
|---|---|
| **IBP** | 174 |
| **10%** | 204 |
| **50%** | 264 |
| **95%** | 347 |
| **FBP** | 359 |

### Diesel Fuel C: Spanish 300 ppm Sulphur

| | |
|---|---|
| **KV@40C (cSt)** | **3.133** |
| **Sulphur content (ppm)** | **300** |
| **Density @15C Kg/litre** | **833.9** |
| **Cloud Point (°C)** | **+1** |
| **IBP (°C)** | **183.7** |
| **10% Recovery** | **224.3** |
| **50% Recovery** | **281** |
| **95% Recovery** | **353.5** |
| **FBP** | **368.9** |

### Diesel Fuel D: Swedish Class 1

| **Test** | **Result** | **Units** |
|---|---|---|
| **Cloud point (Auto)** | **-40** | **°C** |
| **CFPP** | **-40** | **°C** |
| **kV @ 40°C (Auto)** | **1.574** | **cSt** |
| **Density @ 15°C** | **817.6** | **Kg/m³** |
| **Sulphur** | **9** | **mg/kg** |

| **Distillation D86** | | |
|---|---|---|
| **IBP** | **190.9** | **°C** |
| **10%** | **208.8** | **°C** |
| **50%** | **233.3** | **°C** |
| **95%** | **278.8** | **°C** |
| **FBP** | **290.1** | **°C** |

### Diesel Fuel E : Shell Class 1 diesel fuel.

### Diesel Fuel F : a further Class 1 diesel fuel.

### Stability Examples

### Example 4: Investigation of Stability of Colloidal Cerium DPF System in German Low Sulphur (<10 ppm) Diesel Fuels A and B at 80°C

Tables 1 and 2 detail stability results for the colloidal cerium-based DPF additive Eolys^{®}, a cerium containing oil fuel additive marketed by "Rhodia Electronics and Catalysis", a Rhodia Group subsidiary, in low sulphur diesel fuels in the presence of various lubricity improver additive chemistries and in the presence of percentage levels of biodiesel (rapeseed oil methyl ester - RME) respectively. The stability test involved the separate addition of the additive(s) to the respective fuel using normal laboratory blending practices, and thereafter visually observing the blended fuel composition for phase separation and general appearance whilst being stored at 80°C.

The results demonstrate that the cerium-based colloid is fundamentally unstable in low sulphur diesel fuel and evidence of gross phase separation of insoluble precipitates is seen within 1 day during storage at 80°C, even in the absence of the lubricity additive or biodiesel.

The results also show that the RME and the various lubricity improver additives are unlikely to improve the stability of the metal catalyst compound to levels required to ensure safe field operation.

**Table 1. Stability of Colloidal Cerium DPF Additive in German Low Sulphur Diesel Fuel A in the Presence of Representative Types of Lubricity Improver Chemistry**

| **Fuel** | **Eolys^{®} (ppm Ce)** | **Lubricity Improver Chemistry I (ppm)** | **Lubricity Improver Chemistry II (ppm)** | **Lubricity Improver Chemistry III (ppm)** | **Lubricity Improver Chemistry IV (ppm)** | **RME (%)** | **day 1** | **day 2** | **day 4 (end)** |
|---|---|---|---|---|---|---|---|---|---|
| Fuel A | 25 | | | | | | phase sep. | phase sep. | phase sep. |
| Fuel A | 25 | 200 | | | | | phase sep. | phase sep. | phase sep. |
| Fuel A | 25 | 400 | | | | | phase sep. | phase sep. | phase sep. |
| Fuel A | 25 | | 200 | | | | phase sep. | phase sep. | phase sep. |
| Fuel A | 25 | | 400 | | | | phase sep. | phase sep. | phase sep. |
| Fuel A | 25 | | | 200 | | | phase sep. | phase sep. | phase sep. |
| Fuel A | 25 | | | 400 | | | phase sep. | phase sep. | phase sep. |
| Fuel A | 25 | | | | 200 | | phase sep. | phase sep. | phase sep. |
| Fuel A | 25 | | | | 400 | | phase sep. | phase sep. | phase sep. |
| Fuel A | 25 | | | | | 5% | phase sep. | phase sep. | phase sep. |
| Fuel A | 25 | | | | | 30% | hazy | phase sep. | phase sep. |
| RME = Rapeseed Methyl Ester (biodiesel) | | | | | | | | | |

**Table 2. Stability of Colloidal Cerium DPF Additive in German Low Sulphur Diesel Fuel B in the Presence of Representative Types of Lubricity Improver Chemistry**

| **Fuel** | **Eolys^{®} (ppm Ce)** | **Lubricity Improver Chemistry I (ppm)** | **Lubricity Improver Chemistry II (ppm)** | **Lubricity Improver Chemistry III (ppm)** | **Lubricity Improver Chemistry IV (ppm)** | **RME (%)** | **day 1** | **day 2** | **day 4 (end)** |
|---|---|---|---|---|---|---|---|---|---|
| Fuel B | 25 | | | | | | phase sep. | phase sep. | phase, sep. |
| Fuel B | 25 | 200 | | | | | phase sep. | phase sep. | phase sep. |
| Fuel B | 25 | 400 | | | | | phase sep. | phase sep. | phase sep. |
| Fuel B | 25 | | 200 | | | | phase sep. | phase sep. | phase sep. |
| Fuel B | 25 | | 400 | | | | phase sep. | phase sep. | phase sep. |
| Fuel B | 25 | | | 200 | | | phase sep. | phase sep. | phase sep. |
| Fuel B | 25 | | | 400 | | | phase sep. | phase sep. | phase sep. |
| Fuel B | 25 | | | | 200 | | phase sep. | phase sep. | phase sep. |
| Fuel B | 25 | | | | 400 | | phase sep. | phase sep. | phase sep. |
| Fuel B | 25 | | | | | 5% | phase sep. | phase sep. | phase sep. |
| Fuel B | 25 | | | | | 30% | hazy | phase sep. | phase sep. |

### Example 5: Investigation of Stability of Colloidal Cerium DPF Additive in the Presence of Commercial Lubricity Additives in Diesel Fuel C (300 ppm sulphur) and Fuel D (Swedish Class 1, < 10 ppm sulphur) at 80°C

It may be observed from Table 3 that the cerium-based DPF additive (Eolys^{®}) is fundamentally unstable with respect to precipitation/phase separation in the presence of various lubricity additive chemistries in these two different diesel fuels. The same test protocol of separate addition of the additives to the fuel was followed.

This instability of the cerium additive at two concentrations (25 ppm and 250 ppm respectively) is only mitigated in the presence of very high levels (200-1000 ppm) of PIBSA-PAM, a polyisobutenyl succinimide diesel detergent, which contains one imide polar head group per lipophilic chain (ie. not an example according to the invention.)

**Table 3. Stability of Cerium-based DPF Additives at 80°C in the Presence of Some Lubricity Additives in Diesel Fuels C and D**

| **Diesel** | **Eolys^{®} (ppm Ce)** | **Lubricity Improver Chemistry 1 (ppm)** | **Lubricity Improver Chemistry II (ppm)** | **Lubricity Improver Chemistry IV (ppm)** | **PIBSA-PAM (ppm)** | **1 hr.** | **day 1** | **day 4** | **day 5** | **day 7 (end)** |
|---|---|---|---|---|---|---|---|---|---|---|
| Fuel C | 250 | 200 | | | | clear | hazy | phase sep. | phase sep. | phase sep. |
| Fuel C | 250 | 200 | | | 200 | clear | clear | clear | clear | clear |
| Fuel C | 250 | 600 | | | 600 | clear | clear | hazy | hazy | hazy |
| Fuel C | 250 | 600 | | | 800 | clear | clear | clear | clear | slightly hazy |
| Fuel C | 250 | 600 | | | 1000 | clear | clear | clear | clear | clear |
| Fuel C | 25 | | | | | clear | clear | clear | hazy | phase sep. |
| Fuel C | 25 | 200 | | | | clear | hazy | hazy | hazy | phase sep. |
| Fuel C | 25 | 200 | I | | 50 | clear | hazy | hazy | hazy | slightly hazy |
| Fuel C | 25 | 200 | | | 200 | clear | clear | clear | clear | clear |
| Fuel C | 25 | 200 | | | 400 | clear | clear | clear | clear | clear |
| Fuel C | 25 | | | 200 | | hazy | phase sep. | phase sep. | phase sep. | phase sep. |
| Fuel D | 25 | 200 | | | | clear | clear/ hazy? | clear | **sl** phase sep. | phase sep. |
| Fuel D | 25 | | 200 | | | clear | clear | phase sep. | phase sep. | phase sep. |
| Fuel D | 25 | | | 200 | | clear | clear/ hazy? | phase sep. | phase sep. | phase sep. |

### Example 6: Improved Stability of Colloidal Cerium in the Presence of Lubricity Additives when using Stabiliser A of the Present Invention (Part I)

Results given in Table 4 indicate the significantly improved stability of the colloidal DPF system in static storage at 80°C in diesel fuel C in the presence of a lubricity improver when using low levels of the stabiliser molecules of the present invention (Stabiliser A from Example 1).

Between 50-100 ppm of Stabiliser B (Comparative) is able to stabilise the Ce-based composition up to 7 days. Stabiliser A at 50-100 ppm is able to stabilise the similar composition for up to 12 days versus the control samples which exhibit the onset of phase separation from initial sample blending. Both A and B are capable of stabilizing the compositions to such an extent that clear compositions are formed, in some cases for extended periods (and particularly with the stabiliser A). In comparison, low levels of PIBSA-PAM (10-100 ppm), a polyisobutenyl succinimide diesel detergent, which contains one imide polar head group per lipophilic chain, does not provide sufficient stabilization to form clear compositions.

Furthermore, the significantly-improved stability performance of the stabiliser molecule A versus the unreacted starting material, PIBSA, at similar concentration indicates the effectiveness of the present invention in stabilising the cerium colloid in the presence of the lubricity improver additive I.

**Table 4. Improved Stability of Cerium-based DPF Additives at 80°C in the Presence of Lubricity Improver in Diesel Fuel C When Using Stabilising Compositions**

| **Eolys^{®} (ppm Ce)** | **Lubricity Improver Chemistry I (ppm)** | **Stabiliser A (ppm)** | **Stabiliser B (ppm)** | **PIBSA - PAM (ppm)** | **PIBSA (ppm)** | **Day 0** | **Day 3** | **Day 4** | **Day 5** | **Day 6** | **Day 7** | **Day 10** | **Day 11** | **Day 12** | **Day 13** | **Day 14** |
|---|---|---|---|---|---|---|---|---|---|---|---|---|---|---|---|---|
| 25 | 200 | | | | | hazy | PS | PS | PS | PS | PS | PS | PS | PS | PS | PS |
| 25 | 200 | 10 | | | | clear | clear | clear | vs haze | s haze | hazy | v hazy | v hazy | v hazy | sPS | s PS |
| 25 | 200 | 50 | | | | clear | clear | clear | clear | clear | clear | clear | clear | clear | hazy | PS |
| 25 | 200 | 100 | | | | clear | clear | clear | clear | clear | clear | clear | clear | clear | PS | PS |
| 25 | 200 | | 10 | | | hazy | PS | PS | PS | PS | PS | PS | PS | PS | PS | PS |
| 25 | 200 | | 50 | | | clear | clear | clear | clear | vs haze | hazy | v hazy | PS | PS | PS | PS |
| 25 | 200 | | 100 | | | clear | clear | clear | clear | clear | clear | PS | PS | PS | PS | PS |
| 25 | 200 | | | 10 | | v hazy | PS | PS | PS | PS | PS | PS | PS | PS | PS | PS |
| 25 | 200 | | | 50 | | hazy | v hazy | v hazy | v hazy | v hazy | v hazy | s PS | s PS | s PS | s PS | s PS |
| 25 | 200 | | | 100 | | s haze | hazy | hazy | hazy | hazy | hazy | v hazy | v hazy | v hazy | v hazy | v hazy |
| 25 | 200 | | | | 10 | hazy | v hazy | PS | PS | PS | PS | PS | PS | PS | PS | PS |
| 25 | 200 | | | | 50 | clear | clear | clear | s haze | hazy | s PS | PS | PS | PS | PS | PS |
| 25 | 200 | | | | 100 | clear | clear | clear | clear | clear | clear | PS | PS | PS | PS | PS |
| PS = phase separation, v = very, s = slight | | | | | | | | | | | | | | | | |

### Example 7: Improved Stability of Colloidal Cerium in the Presence of Commercial Lubricity Additives When Using Stabilisers of the Present Invention (Part II)

Table 5 gives further stability data for the stabilised Ce colloid, Eolys^{®} in the presence of various lubricity additives.

It may be seen that 35-50 ppm of the stabiliser C (from Example 3) is able to stabilise Eolys^{®} for up to 8 days static storage at 80°C in the presence of large amounts (200 ppm) of lubricity additives I and IV, compared to control samples. The same stabiliser molecule at 50 ppm is able to control the stability of the Ce colloid in the presence of lubricity improver II for up to 5 days.

The various sample controls of Ce colloid and lubricity improver (without stabiliser present) exhibit haze formation and/or phase separation within 1 day. Likewise, the unreacted starting material, PIBSA, shows lesser ability to stabilise the composition against phase separation.

**Table 5. Improved Stability of Cerium-based DPF Additives at 80°C in the Presence of Some Commercial Lubricity Additives When Using Stabilising Compositions**

| **Fuel** | **Eolys^{®} (ppm Ce)** | **Lubricity Improver Chemistry I (ppm)** | **Lubricity Improver Chemistry II (ppm)** | **Lubricity Improver Chemistry IV (ppm)** | **Stabiliser C (ppm)** | **PIBSA (ppm)** | **Day 0** | **Day 1** | **Day 2** | **Day 3** | **Day 4** | **Day 5** | **Day 6** | **Day 7** | **Day 8** |
|---|---|---|---|---|---|---|---|---|---|---|---|---|---|---|---|
| Fuel C | 25 | | | | | | clear | PS | - | - | PS | PS | PS | PS | PS |
| Fuel C | 25 | 200 | | | | | v s haze | hazy | - | - | PS | PS | PS | PS | PS |
| Fuel C | 25 | 200 | | | 10 | | clear | clear | - | - | v hazy | s PS | s PS | PS | PS |
| Fuel C | 25 | 200 | | | 20 | | clear | clear | - | - | clear | clear | hazy | PS | PS |
| Fuel C | 25 | 200 | | | 35 | | clear | clear | - | - | clear | clear | clear | clear | clear |
| Fuel C | 25 | 200 | | | 50 | | clear | clear | - | - | clear | clear | clear | clear | clear |
| Fuel C | 25 | 200 | | | | 10 | v s haze | hazy | - | - | PS | PS | PS | PS | PS |
| Fuel C | 25 | 200 | | | | 20 | clear | v s haze | - | - | PS | PS | PS | PS | PS |
| Fuel C | 25 | 200 | | | | 35 | clear | clear | - | - | clear | v hazy | PS | PS | PS |
| Fuel C | 25 | 200 | | | | 50 | clear | clear | - | - | clear | hazy | PS | PS | PS |
| Fuel C | 25 | | 200 | | | | v hazy | PS | - | - | PS | PS | PS | PS | PS |
| Fuel C | 25 | | 200 | | 10 | | s hazy | hazy | - | - | PS | PS | PS | PS | PS |
| Fuel C | 25 | | 200 | | 20 | | v s haze | v s haze | - | - | PS | PS | PS | PS | PS |
| Fuel C | 25 | | 200 | | 35 | | clear | clear | - | - | v hazy | PS | PS | PS | PS |
| Fuel C | 25 | | 200 | | 50 | | clear | clear | - | - | clear | clear | hazy | PS | PS |
| Fuel C | 25 | | 200 | | | 10 | v hazy | PS | - | - | PS | PS | PS | PS | PS |
| Fuel C | 25 | | 200 | | | 20 | v hazy | PS | - | - | PS | PS | PS | PS | PS |
| Fuel C | 25 | | 200 | | | 35 | hazy | PS | - | - | PS | PS | PS | PS | PS |
| Fuel C | 25 | | 200 | | | 50 | hazy | sPS | - | - | PS | PS | PS | PS | PS |
| Fuel C | 25 | | | 200 | | | clear | PS | - | - | PS | PS | PS | PS | PS |
| Fuel C | 25 | | | 200 | 10 | | clear | clear | - | - | PS | PS | PS | PS | PS |
| Fuel C | 25 | | | 200 | 20 | | clear | clear | - | - | clear | clear | hazy | PS | PS |
| Fuel C | 25 | | | 200 | 35 | | clear | clear | - | - | clear | clear | clear | clear | clear |
| Fuel C | 25 | | | 200 | 50 | | clear | clear | - | - | clear | clear | clear | clear | clear |
| Fuel C | 25 | | | 200 | | 20 | clear | clear | - | - | PS | PS | PS | PS | PS |
| Fuel C | 25 | | | 200 | | 35 | clear | clear | - | - | PS | PS | PS | PS | PS |
| Fuel C | 25 | | | 200 | | 50 | clear | clear | - | - | clear | PS | PS | PS | PS |

### Example 8: Improved Stability of Colloidal Metal Oxide DPF Additives in Fuel D When Using Stabilisers of the Present Invention (Part III)

The results given in the Table 6 indicate the stabilising effect of Stabiliser A from Example 1 on a colloidal mixed cerium oxide and iron oxides additive, 'Eolys^{®} 176', in fuel compositions comprising petroleum-derived diesel fuel D and the biofuel fatty acid methyl ester ('FAME'). In Table 6, the treat rates shown for the CeFe additive are ppm (weight) of total metal in the fuel.

**Table 6**

| **Fuel Blend** | **Additives** | **Stability (days)** |
|---|---|---|
| **5% FAME in fuel D composition** | 10 ppm CeFe | 1 |
| | 10 ppm CeFe + 10 ppm stabiliser A | 1 |
| | 10 ppm CeFe + 25 ppm stabiliser A | 2 |
| | 10 ppm CeFe + 50 ppm stabiliser A | 4 |
| | 10 ppm CeFe + 75 ppm stabiliser A | 5 |
| | 10 ppm CeFe + 100 ppm stabiliser A | 5 |
| | 10 ppm CeFe + 200 ppm LI-V | 1 |
| | 10 ppm CeFe + 200 ppm LI-VI | 1 |
| **2% FAME in fuel D composition** | 10 ppm CeFe | 1 |
| | 10 ppm CeFe + 10 ppm stabiliser A | 1 |
| | 10 ppm CeFe + 25 ppm stabiliser A | 2 |
| | 10 ppm CeFe + 50 ppm stabiliser A | 5 |
| | 10 ppm CeFe + 75 ppm stabiliser A | 12 |
| | 10 ppm CeFe + 100 ppm stabiliser A | 5 |
| | 10 ppm CeFe + 200 ppm LI-V | 1 |
| | 10 ppm CeFe + 200 ppm LI-VI | 1 |

It may be observed that addition of moderate amounts (25-75 ppm) of stabiliser A can markedly improve the stability of the colloidal metallic additive towards phase separation in the presence of the biofuel FAME, compared to the control situation with no stabiliser present.

Moreover, it may be seen that lubricity improver ('LI') chemistry types V and VI* offer no stabilising effect in this system.

### Example 9: Improved Stabilisation Effect from adding Stabiliser of the Present Invention directly into the Colloidal Metal Catalyst Additive Concentrate, prior to addition to the fuel.

Table 7 indicates the excellent stability that may be achieved by adding Stabiliser A from Example 1 directly into a stock solution of Eolys^{®} 176, prior to doping the mixture into either Class 1 diesel fuel E or a fuel composition comprising fuel E and the biofuel fatty acid methyl ester ('FAME').

The results indicate the markedly improved stability that may be achieved from adding the stabiliser moiety directly into the colloidal metal catalyst concentrate prior to doping the mixtures into the fuel. The results may also be compared to those obtained from adding the stabiliser and colloidal DPF additive separately into a fuel composition comprising petroleum-derived diesel fuel and the biofuel fatty acid methyl ester ('FAME') (previous Example 8 above). It is believed that the pre-addition of the stabiliser to the metal additive concentrate causes the re-organisation of the colloidal metal complex in such a way that its oil soluble or oil dispersible character is substantially improved, leading to better performance when subsequently blended into the fuel.

**Table 7**

| **Fuel Blend** | **Additives** | **Stability (days)** |
|---|---|---|
| **Class I diesel fuel** | **Separate blending into fuel** | |
| | 25 ppm Ce | 1 |
| | 10 ppm CeFe | 2 |
| | 25 ppm Ce + 25 ppm Stabiliser A | 4 |
| | 25 ppm Ce + 50 ppm Stabiliser A | 5 |
| | 10 ppm CeFe + 25 ppm Stabiliser A | 5 |
| | 10 ppm CeFe + 50 ppm Stabiliser A | 15 |
| | Pre-blend of stabiliser into concentrate | |
| | 25 ppm Ce + 25 ppm Stabiliser A | 5 |
| | 25 ppm Ce + 50 ppm Stabiliser A | 15 |
| | 10 ppm CeFe + 25 ppm Stabiliser A | 10 |
| | 10 ppm CeFe + 50 ppm Stabiliser A | 15 |
| **2% FAME in fuel composition** | 10 ppm CeFe | 1 |
| | **Pre-blend of stabiliser into concentrate** | |
| | 10 ppm CeFe +25 ppm Stabiliser A | 16 |
| | 10 ppm CeFe +50 ppm Stabiliser A | 5 |
| | 10 ppm CeFe +75 ppm Stabiliser A | 5 |
| | 10 ppm CeFe +100 ppm Stabiliser A | 15 |
| **5% FAME in fuel composition** | 10 ppm CeFe | 1 |
| | **Pre-blend of stabiliser into concentrate** | |
| | 10 ppm CeFe +25 ppm Stabiliser A | 10 |
| | 10 ppm CeFe +50 ppm Stabiliser A | 12 |
| | 10 ppm CeFe +75 ppm Stabiliser A | 16 |
| | 10 ppm CeFe +100 ppm Stabiliser A | 9 |

### Example 10: Engine Test Results: Effect of adding Stabiliser of the Present Invention into a Peugeot 307 Vehicle Fuel Tank

The following Tables 8 and 9 give analytical results for Ce and Fe from samples obtained from the fuel tank of a Peugeot 307 car operated on (i) the mixed cerium and iron additive described in the previous two examples, and (ii) the cerium-only additive described in earlier examples, when used in Fuel F.

This Peugeot car was equipped (as standard factory fit) with a separate on-board tank for storage of a diesel particulate trap additive concentrate, this additive being introduced into the fuel contained in the tank of the car under the control of the on-board engine management system, to achieve the regeneration of the particulate trap. In these tests, the factory-filled additive was replaced by untreated test fuel (ie. containing no additive) to avoid subsequent interference in the test, and the fuel tank filled with test fuel already comprising the mixed cerium and iron additive and stabiliser A previously described, these additives having been added separately to the fuel. The stability of the fuel - additive mixture in the car fuel tank was thereafter assessed by analysis at periodic intervals during the running of the vehicle. At each assessment, sampling from both the top and bottom of the tank fuel gave an indication of the degree of phase separation and/or settlement of the metal additive from the fuel during the normal running of the vehicle.

In each table, the test fuel contained 25 ppm (weight) of stabiliser A and additionally contained a constant level of lubricity additive LI-I.

**Table 8 - mixed cerium and iron additive**

| **Test sample** | **Ce (ppm)** | **Fe (ppm)** |
|---|---|---|
| Initial sample | 0.1 | 0.5 |
| One hour in test, top tank | 6.1 | 2.7 |
| One hour in test, bottom tank | 6 | 2.7 |
| Halfway through test, top tank | 6.1 | 2.8 |
| Halfway through test, bottom tank | 5.8 | 2.7 |
| End of test + 1 hour | 5.2 | 2.4 |
| After fuel drained | 5.3 | 2.5 |

The results in Table 8 demonstrate the maintenance of equivalent levels of metals throughout the fuel tank during the test, consistent with effective stabilization of the metal additive within the fuel.

**Table 9 - cerium-only additive**

| **Test sample** | **Ce (ppm) with Stabiliser A** |
|---|---|
| Initial sample | 21 |
| One hour in test, top tank | 22 |
| One hour in test, bottom tank | 22 |
| Halfway through test, top tank | 21 |
| Halfway through test, bottom tank | 21 |
| End of test + 1 hour | 16 |
| After fuel drained | 22 |

| **Test sample** | **Ce (ppm) without Stabiliser A** |
|---|---|
| Initial sample | 0.5 |
| One hour in test, top tank | 0.5 |
| One hour in test, bottom tank | 0.5 |
| Halfway through test, top tank | 0.5 |
| Halfway through test, bottom tank | 0.5 |
| End of test + 1 hour | 0.5 |
| After fuel drained | 0.5 |

In Table 9, the presence of stabiliser A again leads to maintenance of metal distribution within the tank, in contrast to the control experiment lacking stabiliser A.

## Claims

1. A diesel fuel composition comprising a diesel fuel, a colloidally dispersed or solubilised metal catalyst compound for diesel particulate trap regeneration and 10 to 1,000 ppm of an oil soluble or oil dispersible organic compound having a lipophilic hydrocarbyl chain having attached directly thereto at least two contiguous polar head functional groups, wherein the metal catalyst compound consists of cerium or iron oxides or mixtures thereof, and wherein the organic compound is represented by the generalised formula A-C-B, where C represents a hydrocarbyl chain of Mn (number average molecular weight) of 200 - 4,000, and A and B represent at least two contiguous carboxylate residues attached directly to one end of the lipophilic C chain, being either groups of the formula -COOH or ionized as -(COO⁻)ₙMⁿ⁺ where M is a quaternary ammonium cation.

2. The composition of claim 1 wherein the hydrocarbyl chain is a polyisobutenyl group of Mn 200 - 4,000.

3. The composition of claim 2 wherein the organic compound is polyisobutenyl succinic acid wherein the polyisobutenyl group has a Mn of 1,000 or 450.

4. The composition of any preceding claim further comprising a lubricity additive.

5. The composition of any preceding claim further comprising a cold flow additive.

6. The composition of any preceding claim further comprising a diesel detergent additive.

7. The composition of any preceding claim wherein the diesel fuel contains 2000 ppm or less of sulphur.

8. A diesel fuel additive concentrate composition comprising a carrier fluid, the colloidally dispersed or solubilised metal catalyst compound defined in claim 1, 3 to 75 wt. % of a stabiliser additive comprising the oil soluble or oil dispersible organic compound defined in any of claims 1 to 3, and one or more other fuel additives selected from other lubricity-enhancing compounds; cold flow improvers such as ethylene-unsaturated ester copolymers, hydrocarbon polymers, polar nitrogen compounds, alkylated aromatics, linear polymer compounds and comb polymers; detergents; corrosion inhibitors; dehazers; demulsifiers; metal deactivators; antifoaming agents; combustion improvers such as cetane improvers; package compatibilisers; reodorants; metallic-based additives such as metallic combustion improvers; dyes; bacteriostatic agents; gum inhibitors; upper cylinder lubricants and anti-icing agents and antioxidants.

9. The use, in a diesel fuel composition comprising a diesel fuel and the colloidally dispersed or solubilised metal catalyst compound defined in claim 1, of the oil soluble or oil dispersible organic compound defined in any of claims 1 to 3, to reduce the tendency of the diesel fuel and the colloidally dispersed or solubilised metal catalyst compound to form separate phases within the diesel fuel composition over time.

10. The use of the oil soluble or oil dispersible organic compound defined in any of claims 1 to 3 in an additive concentrate comprising the metal catalyst compound defined in claim 1 to improve the colloidal dispersability or solubility of the metal catalyst compound in diesel fuel.

11. A process for enhancing the oil dispersibility or solubility of the metal catalyst compound defined in claim 1, comprising the addition thereto of the oil soluble or oil dispersible organic compound defined in any of claims 1 to 3 to a diesel fuel composition comprising a diesel fuel and the metal catalyst compound.

## Patentansprüche

1. Dieselkraftstoffzusammensetzung, die Dieselkraftstoff, kolloidal dispergierte oder löslich gemachte Metallkatalysatorverbindung für die Regenerierung von Dieselkraftstoffpartikelabscheidern und 10 bis 1000 ppm öllösliche oder öldispergierbare organische Verbindung umfasst, die eine lipophile Kohlenwasserstoffkette aufweist, an der mindestens zwei benachbarte polare funktionale Kopfgruppen direkt gebunden sind, wobei die Metallkatalysatorverbindung aus Cer- oder Eisenoxiden oder Mischungen davon besteht, und wobei die organische Verbindung durch die verallgemeinerte Formel A-C-B dargestellt ist, wobei C eine Kohlenwasserstoffkette mit Mn (durchschnittliches Molekulargewicht (Zahlenmittel)) von 200 bis 4000 darstellt, und A und B mindestens zwei benachbarte Carboxylatreste darstellen, die direkt an ein Ende der lipophilen C-Kette gebunden sind, die entweder als Gruppen mit der Formel -COOH oder ionisiert als -(COO⁻)ₙMⁿ⁺ vorliegen, wobei M ein quartäres Ammoniumkation ist.

2. Zusammensetzung nach Anspruch 1, bei der die Kohlenwasserstoffkette eine Polyisobutylengruppe mit Mn 200 bis 4000 ist.

3. Zusammensetzung nach Anspruch 2, bei der die organische Verbindung Polyisobutylenbernsteinsäure ist, wobei die Polyisobutylengruppe ein Mn von 1000 oder 450 aufweist.

4. Zusammensetzung nach einem der vorhergehenden Ansprüche, die ferner Schmieradditiv umfasst.

5. Zusammensetzung nach einem der vorhergehenden Ansprüche, die ferner Kaltfließadditiv umfasst.

6. Zusammensetzung nach einem der vorhergehenden Ansprüche, die ferner Diesel-Detergensadditiv umfasst.

7. Zusammensetzung nach einem der vorhergehenden Ansprüche, bei der der Dieselkraftstoff 2000 ppm oder weniger Schwefel enthält.

8. Additivkonzentrat-Zusammensetzung für Dieselkraftstoff, das Trägerflüssigkeit, die kolloidal dispergierte oder löslich gemachte Metallkatalysatorverbindung wie in Anspruch 1 definiert und 3 bis 75 Gew.-% Stabilisatoradditiv umfasst, das die öllösliche oder öldispergierbare organische Verbindung wie in einem der Ansprüche 1 bis 3 definiert umfasst und einen oder mehrere Kraftstoffadditive ausgewählt aus anderen schmierfähigkeitsverbessernden Verbindungen; Kaltfließverbesserer wie Ethylen-ungesättigte Ester-Copolymere, Kohlenwasserstoffpolymere, polare Stickstoffverbindungen, alkylierte Aromaten, lineare Polymerverbindungen und Kamm-Polymere; Detergenzien; Korrosionsschutzmittel; Enttrübungsmittel; Metalldeaktivatoren; Entschäumer; Verbrennungsverbesserer wie Cetanverbesserer; Kompatibilisierungsmittel; Geruchsüberdecker; Additive auf Metallbasis wie metallische Verbrennungsverbesserer; Farbstoffe; bakteriostatische Mittel; Gummihemmer; Schmiermittel für den oberen Zylinder und Anti-Eis-Mittel und Antioxidantien.

9. Verwendung der öllöslichen oder öldispergierbaren organischen Verbindung wie in einem der Ansprüche 1 bis 3 definiert in einer Dieselkraftstoffzusammensetzung, die Dieselkraftstoff und die kolloidal dispergierte oder löslich gemachte Metallkatalysatorverbindung wie in Anspruch 1 definiert umfasst, um die Tendenz des Dieselkraftstoffs und der kolloidal dispergierten oder löslich gemachten Metallkatalysatorverbindung zu verringern, über die Zeit innerhalb der Dieselkraftstoffzusammensetzung separierte Phasen zu bilden.

10. Verwendung der öllöslichen oder öldispergierbaren organischen Verbindung wie in einem der Ansprüche 1 bis 3 definiert in einem Additivkonzentrat, das die Metallkatalysatorverbindung wie in Anspruch 1 definiert umfasst, um die kolloidale Dispergierbarkeit oder Löslichkeit der Metallkatalysatorverbindung in Dieselkraftstoff zu verbessern.

11. Verfahren zur Verbesserung der Öldispergierbarkeit oder -löslichkeit einer Metallkatalysatorverbindung wie in Anspruch 1 definiert, bei welchem Verfahren die öllösliche oder öldispergierbare organische Verbindung wie in einem der Ansprüche 1 bis 3 definiert zu einer Dieselkraftstoffzusammensetzung, die Dieselkraftstoff und die Metallkatalysatorverbindung umfasst, hinzugegeben wird.

## Revendications

1. Composition de carburant diesel comprenant un carburant diesel, un composé catalyseur métallique dispersé ou solubilisé colloïdalement pour la régénération d'un piège à particules diesel et 10 à 1000 ppm d'un composé organique soluble dans l'huile ou dispersible dans l'huile ayant une chaîne hydrocarbyle lipophile y ayant directement fixé au moins deux groupes fonctionnels de tête polaire contigus, dans laquelle le composé catalyseur métallique est constitué d'oxydes de cérium ou de fer ou de leurs mélanges, et dans laquelle le composé organique est représenté par la formule généralisée A-C-B, où C représente une chaîne hydrocarbyle de Mn (poids moléculaire moyen en nombre) de 200 à 4000, et A et B représentent au moins deux résidus de carboxylate contigus fixés directement à une extrémité de la chaîne C lipophile, étant soit des groupes de la formule -COOH, soit ionisés comme -(COO⁻)ₙMⁿ⁺ où M est un cation ammonium quaternaire.

2. Composition selon la revendication 1 dans laquelle la chaîne hydrocarbyle est un groupe polyisobutényle de Mn 200 - 4000.

3. Composition selon la revendication 2 dans laquelle le composé organique est de l'acide polyisobuténylsuccinique dans laquelle le groupe polyisobutényl a un Mn de 1000 ou 450.

4. Composition selon l'une quelconque des revendications précédentes comprenant en outre un additif de lubrification.

5. Composition selon l'une quelconque des revendications précédentes comprenant en outre un additif d'écoulement à froid.

6. Composition selon l'une quelconque des revendications précédentes comprenant en outre un additif détergent diesel.

7. Composition selon l'une quelconque des revendications précédentes, dans laquelle le carburant diesel contient 2000 ppm ou moins de soufre.

8. Composition concentrée d'additif de carburant diesel comprenant un fluide porteur, le composé catalyseur métallique dispersé ou solubilisé colloïdalement défini selon la revendication 1, 3 à 75 % en poids d'un additif stabilisant comprenant le composé organique soluble dans l'huile ou dispersible dans l'huile défini selon l'une quelconque des revendications 1 à 3, et un ou plusieurs autres additifs de carburant choisis parmi d'autres composés d'amélioration de la lubrification ; des agents d'amélioration de l'écoulement à froid tels que les copolymères d'ester insaturés d'éthylène, polymères d'hydrocarbures, composés d'azote polaire, aromatiques alkylés, composés polymères linéaires et polymères peignés ; détergents ; inhibiteurs de corrosion ; dégazeurs ; désémulsifiants ; désactivateurs métalliques ; agents antimousses ; agents d'amélioration de la combustion tels qu'un améliorant de cétane ; compatibilisateurs d'emballage ; réodorants ; additifs à base métallique tels que les agents d'amélioration de la combustion métallique ; colorants ; agents bactériostatiques ; inhibiteurs de gomme ; lubrifiants de cylindre supérieur et agents antigel et antioxydants.

9. Utilisation, dans une composition de carburant diesel comprenant un carburant diesel et le composé catalyseur métallique dispersé ou solubilisé colloïdalement défini selon la revendication 1, du composé organique soluble ou dispersible dans l'huile défini selon l'une quelconque des revendications 1 à 3, pour réduire la tendance du carburant diesel et du composé catalyseur métallique dispersé ou solubilisé colloïdalement à former des phases distinctes au sein de la composition de carburant diesel au fil du temps.

10. Utilisation du composé organique soluble ou dispersible dans l'huile défini dans l'une quelconque des revendications 1 à 3 dans un concentré d'additif comprenant le composé catalyseur métallique défini dans la revendication 1 pour améliorer la dispersibilité ou la solubilité colloïdale du composé catalyseur métallique dans le carburant diesel.

11. Procédé d'amélioration de la dispersibilité ou de la solubilité dans l'huile du composé catalyseur métallique défini selon la revendication 1, comprenant l'ajout du composé organique soluble dans l'huile ou dispersible dans l'huile défini selon l'une quelconque des revendications 1 à 3 à une composition de carburant diesel comprenant un carburant diesel et le composé catalyseur métallique.
